

Aug. 29, 1972

L. HÄRTMANN

**3,687,712**

## WEAR RESISTANT NONWOVEN FABRIC

Filed April 16, 1968



**INVENTOR**

DR. LUDWIG HARTMANN  
BY

Burgess, Linklater & Sprung  
ATTORNEYS.

**1****3,687,712****WEAR RESISTANT NONWOVEN FABRIC**Ludwig Hartmann, Blutenweg 1,  
Oberflockenbach, Germany

Filed Apr. 16, 1968, Ser. No. 721,648

Claims priority, application Japan, Feb. 10, 1968,  
43/8,322

Int. Cl. C23f 17/00; D04h 3/03

U.S. Cl. 117—68

6 Claims

**ABSTRACT OF THE DISCLOSURE**

Nonwoven fabric made up of substantially continuous filaments having a relatively low denier and impregnated with binder material concentrated at both major surfaces thereof. Method of making such bonded fabric by introducing binder in the form of a fluid foam onto both surfaces of a nonwoven fleece, preferably sequentially, and drying such binder in a manner such that the binder particles tend to migrate and concentrate at the fabric surface.

It is known that non-woven fabrics can be made of staple fiber of a variety of kinds. It is further known that nonwoven fabrics can be made of substantially continuous filaments.

In the manufacture of nonwoven fabrics which are to be used as underwear or outerwear materials, the most important requirements of the fabric are good mechanical strength and good wear resistance. Next, after these properties, it is necessary that the fabrics possess good breathability. Experiments in the manufacture of materials for longwearing outer garments from staple fibers, especially cellulosic and synthetic organic polymeric fibers, have resulted in a failure to produce satisfactory fabrics for such garments because the fabrics have been insufficient as regards their wear and strength characteristics, since such characteristics could not be satisfied by non-woven fabrics made from short fibers or staple fibers. Furthermore, it has developed that nonwoven batting of this kind does not have adequate wrinkle resistance so that garments made from such fabrics become unsightly after a short period of wear. In addition to short fiber length, a part of the difficulty has also been attributed to the inadequate adhesion of binding substance to the finish-coated staple fibers of the prior art. This inadequate adhesion between the binding agent and the fiber system has not been as apparent or detrimental in the previous uses of such batting as it has been in the case of an outer garment which is subjected to considerable stress during wearing.

Similar difficulties have been observed with a nonwoven fabric consisting of continuous fibers, such as one produced according to British Pat. 1,055,187, which is of continuous filaments impregnated in the usual manner with binding agents for the purpose of obtaining a stable nonwoven fabric from the relatively loose continuous filament batts.

It is therefore an object of this invention to provide a novel nonwoven fabric which avoids the difficulties of the prior art.

It is another object of this invention to provide a novel method of making such novel fabric.

Other and additional objects of this invention will become apparent from a consideration of this entire specification, including the drawing and claims hereof.

In accordance with, and fulfilling these objects, one aspect of this invention resides in a novel nonwoven fabric comprising substantially continuous filaments in the shape of a fabric having bonding agent impregnated into said fabric predominantly at the major surfaces thereof.

**2**

The wear-resistant nonwoven fabric of this invention have a substantially uniform batt structure consisting of thin, continuous polymer filaments which are bonded together with about 25 to 60% and, preferably, 40 to 50% binding agent, which batts are characterized in that over 60% of all filaments thereof have a titer between 0.4 and 1.2 denier, and in that the binding agent is concentrated at the surfaces of the nonwoven fabric.

The important thing is, among others, that continuous filament batts are twice impregnated, preferably with polyacrylic binding agents. The underwear or outerwear material thus obtained shows, not only good air and water-vapor permeability, but also high tear and wear resistance.

These qualities are the consequence of the fact that, for one thing, the continuous filaments of the batt are, in contrast to batts to carded staple fibers, substantially free of any kind of surface finishing agents, lubricants or other such substances on the surfaces thereof.

It has developed that, in the manufacture of outerwear types of unwoven fabrics having high wear resistance, an especially high adherence of binding agents is necessary. This especially high adherence can be achieved substantially only if the filaments are free of any secondary surface-modifying substances.

The continuous filament batts serving as starting material for the fabric of this invention are particularly suitable for the manufacture of outerwear types of nonwoven fabrics if they are made of especially fine filaments. With uniform weight per unit of area and with the uniform battting achieved according to the above mentioned method of producing continuous filament battings, the fabric structure becomes increasingly dense as the filament thickness is reduced. It is apparent that the filament fineness thus has a decisive influence on the breathability of the nonwoven fabric. If the filament diameters are too great, an excessively open structure is produced at a given weight per unit of area, giving an insufficient degree of coverage. It has been found that spun continuous filament battting produced according to the above-referred British patent are particularly well-suited for the manufacture of outerwear types of products if their fiber content consists of more than about 60% of filaments having a titer of less than about 1.2 denier and more than about 0.4 denier. It is not absolutely necessary for the entire amount of the fibers to be within this range of titers. A small amount, e.g. about 5% of the filaments, may have a titer of less than about 0.4 denier. Furthermore, a larger percentage—up to about 40—may have still coarser titers of up to about 3 denier, if special characteristics are required.

In order to produce such mixed filament fabrics, coarse filaments can be spun into the fabrics, as effect filaments, without difficulty by mixed spinning, such as is described in the referred to British patent, by having adjacent nozzles eject different kinds of filaments. These different filaments are worked into a coherent battting by oscillating the guiding ducts.

As previously mentioned, the porosity of the fabric being made has an influence on its subsequent properties, and the porosity is adjustable according to the titer make-up of the fibers of the non-woven batting material. In order to measure the influence of the porosity of the fiber batting structure on the porosity of the end product bonded fabric, one may have recourse to the measurement of air permeability under standardized conditions (DIN 53,887). A filament batt manufactured according to the British patent from nylon 6 with an average titer of 0.8 denier, and having a weight of 100 g./m.<sup>2</sup>, has an air permeability of 1040 l./sec./m.<sup>2</sup> (at 10 mm. water column ΔP), and if the weight is 50 g./m.<sup>2</sup>, the permeability is 1560 l./sec./m.<sup>2</sup> under the same conditions.

In order to use this still loose battting, consisting of continuous filaments, for the manufacture of a wear-

resistant nonwoven fabric, the filaments must then be cemented at their intersections. However, it has developed that, in order to manufacture outer wear-type unwoven fabrics from substantially continuous filaments that have been made according to the prior art, an impregnation method must be used in which the binding agent is concentrated at the two major surfaces of the batting.

It is therefore another aspect of this invention to provide a novel process of producing the above-defined nonwoven fabric, which process comprises forming a nonwoven batting of continuous filaments, preferably by the process of the above mentioned British patent but not necessarily restricted to such preparative technique; preparing a fluid-form foam of the bonding agent, desired to be used in making the fabric of this invention; applying the fluid foam to one major surface of the nonwoven batting; drying such impregnated foam in such manner that the binder particles tend to migrate to and concentrate at the major surface which was impregnated with the fluid foam; and repeating the fluid-foam binder impregnation and drying on the other major surface of the partially bonded nonwoven batting.

It will be appreciated that the particles of binding agent are concentrated away from the core of the nonwoven batt and towards the two major surfaces thereof but that enough binder is also in the middle of the fabric to prevent delamination. It should be noted that, since the dispersed binder particles first deposit themselves along the filament axes and especially at the filament intersections, the organization of the batting filamentary structure of the nonwoven fabric subsequently obtained, which structure is permeated with capillaries.

It has been determined that concentrations of the binding agent in the impregnating foam-form fluid of up to a maximum of 20% are usable for the manufacture of the fabric according to the invention, with concentrations of 6% to 10% being preferred. In the case of higher impregnating liquid concentration, the wear-resistance of the nonwoven fabric diminishes rapidly. This can be explained by the fact that, after the complete impregnation of the loose batt, a migration of water towards both surfaces takes place in the drying, causing a certain amount of the binding agent particles to be thus carried toward the surface before coagulation thereof is complete. This percentage increases as the dilution increases. That this phenomenon is very important can also be seen in the fact that the addition of a larger amount of wetting agents during the impregnation facilitates manufacture of the nonwoven fabrics in accord with the invention. The increased addition of wetting agents stabilizes the foam-form dispersion and promotes migration of binder particles to the surface.

Furthermore, the weight ratio of the binding agent to the filament weight is important. It has been found that the weight of the binding agent should not be less than about 30% of the fabric final weight, nor more than about 50% of the fabric final weight. Binding-agent contents of 40 to 45%, based upon the final weight of fabric, are preferred. If a spun batting is impregnated with about 44% of a polyacrylic dispersion described further below, the fabric has an air permeability of 940 l./sec./m.<sup>2</sup> for a final weight of 100 g./m.<sup>2</sup> and an average titer of 0.8 denier; a similar fabric of 50 g./m.<sup>2</sup> has an air permeability of 1670 l./sec./m.<sup>2</sup>, i.e., the combined fiber and binding agent has porosities on the same order of magnitude as the plain fiber material, for comparable final weights.

As already mentioned, both surfaces of the nonwoven fabric should contain a concentration of binding agent. This can best be achieved by a two-step impregnation, such as set forth generally above. It is preferred that the impregnation should be carried out with certain rules being observed.

In order to obtain good adherence of the binding agent to the filamentary structure, the filaments should be as free as possible from any kind of coatings of other sub-

stances. The impregnating process should be performed in such a manner that both sides of the web of material will contain substantially equal amounts of binding agent, care being taken to see that, after the first surface has set, the other side is not too heavily loaded with the binder of the first impregnation process. In practice it has developed that, in order to achieve optimum adherence of the binding agent, the filaments must be substantially free of foreign substances. If a two-step impregnation is performed, in which first one and then the other side is set, traces of binding agent from the first impregnation, which might penetrate through to the opposite side, are foreign substances insofar as the second impregnation is concerned. This can be explained by the fact that these particles coagulate and crosslink to a certain extent during the drying process so that they are both chemically and physically different from the fresh impregnation mixture that is to be applied. Therefore, care must be taken to see that each impregnation mixture is applied to a loose, fibrous surface. This process can be performed particularly well if binding agents are used in the form of foam because the density and thickness of the foam permit the penetration of the fiber structure to be well-controlled. In the first impregnation, a foam of such a nature is applied that it penetrates barely beyond the center of the fiber material so that the second impregnation of the opposite side can be applied to clean, so-called "native," fibers. If this foamed dispersion also has a low contents of solids, a large percentage of the binding agent particles can migrate toward the surface during drying, and thus produce a very good wear resistance.

In the manufacture of nonwoven batting according to the invention, suitable for use in outerwear, it proves to be particularly desirable to impregnate these battings made of low denier polyamide filaments with polyacrylates containing copolymerized acrylonitrile in addition to a cross-linking component, such as N-methylol acrylamide. The polyacrylates must in any case be chemically cross-linked in order to achieve good washability and dry-cleanability.

The penetrating ability of the impregnating foams must be adapted to the specific weight of the filamentary batting. This is achieved by variations of the foam density and variations of the solids content of the impregnation mixture. It has developed that, for filamentary battings made of nylon 6, as described above, and having the above titer compositions, the following foam adjustments are necessary:

|    | Filamentary batt weight, g./m. <sup>2</sup> | Foam weight, g./l. |
|----|---------------------------------------------|--------------------|
| 20 |                                             | 70-110             |
| 30 |                                             | 115-150            |
| 40 |                                             | 150-230            |

If the foam weight is varied within these limits on the basis of its solids content, and the solids content is from 5 to 20%, the generation of the foam will take place in the manner that is correct for the final solidification.

Understanding of this invention will be facilitated by reference to the accompanying drawing, which is a schematic flow diagram of the process described herein.

By means of a known spinning apparatus, for example, from British Pat. 1,055,187, a molten mass of polycaprolactam at a temperature of 230° C. is spun into filaments 2. The spinning apparatus has several nozzles with 160 orifices 3 having a diameter of 400 microns. The space between spinneret orifice amounted to 2 mm. Hot air at a temperature of 240° C. was blasted at a velocity of 200 m./sec. from the two air slits 4 running parallel to the spinneret holes. The row of filaments emerging from the holes, after traveling a distance of 45 mm., entered into a duct 5 together with the "air ribbons" flowing from the air slits, while a cooling took place so that the air temperature upon leaving the bottom end of the air duct amounted to only 66° C., at a room temperature of 40° C.

After the row of filaments had been deposited on the receiving surface 6, the diameter of the filaments was de-

terminated, and the following filament-size distribution was found:

1.5% had a diameter of less than 0.4 denier  
84% had a diameter between 0.41 and 1.2 denier  
14.5% had a diameter between 1.2 and 1.8 denier.

The weight amounted to 28 g./m.<sup>2</sup>, and the air permeability was 1700 l./sec./m.<sup>2</sup>.

The batting 7 was then impregnated in a two-step process with a copolymer of n-butyl acrylate and N-methylolacrylamide incorporating up to 10% of copolymerized acrylonitrile (e.g., Acronal KR 2249).

First a foam of the above binding agent 8 was applied to one side of the batting in such quantities that the binding agent absorption after passage through a set of rollers amounted to about 11 g./m.<sup>2</sup>. The foam had a content of 10% solids.

The solid itself consisted of:

|                                               | Parts |
|-----------------------------------------------|-------|
| Polyacrylate with copolymerized acrylonitrile | 96    |
| Polyvinyl alcohol                             | 1     |
| Ammonoxalate                                  | 6     |
| Silastan (wetting agent)                      | 6     |

A foam of 120 g. per liter was prepared by mixing in air with an Oaks mixer.

In this foam impregnation, the roller pressure is to be adjusted so that the binding agent does not penetrate to the bottom side.

Then the batting thus impregnated is carried into a drying chamber 9 where air at 120° C. is blown onto the surface of the batting on which the foam had been applied. During the drying, a migration of the binding agent to the hotter surface takes place. In other words, a concentration of the binding agent takes place at the surface to which the foam has just been applied. If during the impregnation an amount of binding agent should have penetrated through to the bottom surface, it would largely migrate back again during the drying. In this manner the bottom side remains loose-fibered.

After leaving the dryer the web 10 of material is inverted and the impregnation process is repeated under the same conditions. The double impregnated web 11 is dried again at 120° C. and heated for another three minutes at 150° C. in a dryer 12 to thoroughly condense the binding agent.

The resulting nonwoven fabric manufactured in this manner weighed 50 g./m.<sup>2</sup> and had good resistance to washing and dry-cleaning. Its air permeability amounted to 1650 l./sec./m.<sup>2</sup> at 10 mm. water column ΔP.

What is claimed is:

1. A wear resistant nonwoven textile fabric comprising a web of varying denier substantially continuous filaments having at least about 60% of said filaments with deniers of 0.4 to 2.0 bonded together throughout at the intersections thereof with an acrylic bonding agent comprising about 25 to 60 weight percent of said fabric, which bond-

ing agent is concentrated at and substantially adjacent to the two major surfaces thereof, and is also present in the middle of the fabric to an extent sufficient to prevent delamination of said fabric.

5 2. Fabric as claimed in claim 1, wherein said bonding agent comprises about 40 to 50 weight percent thereof.

3. Fabric as claimed in claim 1, wherein said bonding agent is a cross-linked polymer of acrylonitrile, n-butylacrylate and N-methylolacrylamide.

10 4. Fabric claimed in claim 1, wherein said filaments are polyamide.

5. Fabric as claimed in claim 1, wherein said filament size distribution is up to about 5% less than about 0.4 denier; up to about 40% about 1.2 to 3 denier; and the remainder about 0.4 to 1.2 denier.

15 6. Process of producing a nonwoven fabric as claimed in claim 1, comprising; preparing a non-woven web of thermoplastic substantially continuous filaments; preparing a fluid-foam impregnant composition comprising an

20 aqueous dispersion of an acrylic resin having a solids content of up to about 20 weight percent; coating said fluid foam onto a first major surface of said non-woven web and impregnating such foam into said web; heating said coated and impregnated web to a temperature and for a

25 time sufficient to substantially remove the liquid portion of the impregnant, to cause said resin to migrate toward said heat and to deposit said resin substantially at and adjacent to said first major surface; coating the second major surface of said nonwoven web with a second aliquot

30 of said fluid foam and impregnating such foam into said web; and heating said second coated and impregnated web to a temperature and for a time sufficient to substantially remove the liquid portion of the impregnant, to cause said resin to migrate toward said heat and to deposit said

35 resin substantially at and adjacent to said second major surface while retaining enough bonding agent in the middle of the fabric to prevent delamination thereof.

#### References Cited

##### UNITED STATES PATENTS

|              |         |                |           |
|--------------|---------|----------------|-----------|
| 3,030,232    | 4/1962  | Morgenstern    | 117—68 X  |
| 3,323,959    | 6/1967  | Kreckl         | 117—140 A |
| 3,471,315    | 10/1969 | Böe et al.     | 161—164 X |
| 45 2,972,554 | 2/1961  | Muskat et al.  | 161—157 X |
| 3,274,046    | 9/1966  | Shannon et al. | 161—157 X |

##### FOREIGN PATENTS

|           |        |                |
|-----------|--------|----------------|
| 1,055,187 | 1/1967 | Great Britain. |
|-----------|--------|----------------|

50 ROBERT F. BURNETT, Primary Examiner

R. L. MAY, Assistant Examiner

##### U.S. CL. X.R.

55 117—140 A, 161 UN; 156—167, 181; 161—140, 164